

# United States Patent Office.

WILLIAM ENNIS, OF PHILADELPHIA, PENNSYLVANIA.

*Letters Patent No. 97,897, dated December 14, 1869.*

## IMPROVEMENT IN THE MANUFACTURE OF IRON AND STEEL.

The Schedule referred to in these Letters Patent and making part of the same

*To all whom it may concern:*

Be it known that I, WILLIAM ENNIS, of the city of Philadelphia, in the county of Philadelphia, and State of Pennsylvania, have discovered a new and useful Improvement in the Manufacture of Iron and Steel, of which the following is a clear and exact description.

My invention consists in forcing hydrogen, separate and free as possible from oxygen, through molten metal, for the purpose of taking up, in its passage through the molten metal, the carbon, sulphur, phosphorus, arsenic, &c., therein contained, forming carburetted hydrogen, sulphuretted hydrogen, phosphoretted hydrogen, &c., which, as they issue from the mass of molten metal, are combined with a current or currents of atmospheric air, or oxygen, introduced over the molten metal, within a chamber of reflecting character, for the purpose of producing the combustion of the carburetted hydrogen, sulphuretted hydrogen, phosphoretted hydrogen, &c., and retaining the mass in its proper fluid state.

This method of treating the molten metal, though designed to effect a similar general purpose of converting the molten mass into refined iron, radically differs from what is known as the Bessemer process of forcing oxygen, or oxygen and hydrogen, alternately or combined, through the molten mass, which not only takes up carbon, but, owing to the affinity of oxygen for iron, destroys or injuriously affects it.

This is not the case when hydrogen alone is

forced from below, in a diffused manner, through the molten metal, while the carburetted hydrogen, sulphuretted hydrogen, and phosphoretted hydrogen formed thereby, are ignited as they emerge above the surface of the mass, where the combustion is kept up by the introduction of a stream or streams of atmospheric air, or oxygen, over and above, in contradistinction to up and through the molten metal, which combustion, taking place within a chamber or arch of reflecting character, produces the requisite intensity of heat over the mass, in addition to which the passage of hydrogen through molten metal, portions of which hydrogen combine with the metal, giving it a character which it did not before possess.

What I claim as my invention, and desire to secure by Letters Patent, is—

In the manufacture of iron and steel, subjecting the mass of molten metal to the action of hydrogen-gas alone, forced up through the mass, in combination with a current or currents of atmospheric air, or oxygen, introduced over the molten metal within a chamber of reflecting character, producing combustion of the carburetted hydrogen, sulphuretted hydrogen, phosphoretted hydrogen, &c., above the metal, substantially as and for the purpose specified.

WILLIAM ENNIS.

Witnesses:

W. M. P. SHATTUCK,  
C. C. SELDEN.